

# United States Patent Office.

CHARLES TOPPAN, OF WAKEFIELD, MASSACHUSETTS.

Letters Patent No. 89,094, dated April 20, 1869.

## IMPROVED MODE OF TREATING PAPER AND OTHER FABRICS TO RENDER THEM WATER-PROOF.

The Schedule referred to in these Letters Patent and making part of the same.

*To all whom it may concern:*

Be it known that I, CHARLES TOPPAN, of Wakefield, in the county of Middlesex and State of Massachusetts, have invented a new and useful Mode of Treating Paper and other Fabrics, to render them Water-proof; and I hereby declare that the following is a full and exact description thereof.

My invention consists in preparing paper, cloth, felting, or textile fabrics of any kind, cork, sponge, leather, and other similar porous substances, and articles made thereof, especially wrapping-paper, bank-notes, envelopes, paper collars, garments, gloves, hats, umbrella-coverings, labels, tags, &c., so as to render the same impervious to water, by applying thereto paraffine dissolved in naphtha, benzine, or other suitable solvents.

To enable others skilled in the art to understand and use my invention, I will proceed to describe the manner in which I have carried it out.

I prepare a solution of paraffine by dissolving paraffine in pure naphtha, that is, naphtha free from any oily or greasy matter, or naphtha that will not stain letter-paper when dipped into it and dried.

The paraffine should be cut into small pieces, and put into the naphtha in an easily and tightly-closed vessel, and should then be well shaken or agitated. In this way, a saturated cold solution may be quickly obtained without the use of heat.

It is best to use an excess of paraffine in the naphtha, so as to have a saturated solution at about 70° Fahrenheit.

The fabrics or articles to be prepared are dipped

into this solution, and, if necessary, are allowed to remain there some time. The length of time will depend upon the thickness and porosity of the material, but should be sufficient to allow the solution to either penetrate thoroughly, if so desired, or the time may be so short as to allow the solution to penetrate only a short distance from the surface.

The fabrics or articles thus treated are then removed, and dried by artificial or natural heat, or in a current of air, when the naphtha evaporates and leaves the paper, cloth, or other article, filled with paraffine, and impervious to water.

I have found naphtha (including benzine and benzole) of very light gravity to be the most suitable solvent.

The best results are obtained by the use of refined paraffine, but crude paraffine may be used for many articles.

I do not claim the preparation of paper, or cloth, or other fabric, by the application of paraffine in a melted state.

What I claim as my invention, and desire to secure by Letters Patent, is—

The treatment of paper, cloth, cork, sponge, leather, and other similar felted or textile fabrics and porous substances, or articles made therefrom, by the application thereto of paraffine in solution, substantially as described, for the purpose set forth.

CHARLES TOPPAN.

Witnesses:

CHARLES A. PHILLIPS,  
N. W. STEARNS.